

## UNITED STATES PATENT OFFICE.

HEINRICH HELBING, OF LONDON, ENGLAND.

## CORK.

SPECIFICATION forming part of Letters Patent No. 734,551, dated July 28, 1903.

Application filed May 10, 1902. Serial No. 106,816. (No specimens.)

*To all whom it may concern:*

Be it known that I, HEINRICH HELBING, consulting chemist, of 63 Queen Victoria street, London, England, have invented certain new and useful Improvements in Corks, of which the following is a specification.

This invention relates to improvements in corks.

It is well known that wine and other potable liquids stored in bottles and the like with cork stoppers frequently exert a gradual dis-solvent or deteriorating effect upon the cork, whereby the cork itself becomes softened and rotten or the liquid acquires a corky taste or sometimes a bad color. It has been attempted to remedy these defects by coating the surface of the cork with paraffin or with solutions of caoutchouc, nitrocellulose, or the like; but it has been found that the employment of these protective layers is in practice accompanied by serious disadvantages.

I have now discovered that the endurance and impermeability of the cork may be greatly increased without material loss of elasticity by impregnating the cork with casein or other albumen capable of forming soluble salts with alkalies and fixing the albumen preferably with formic aldehyde. The corks may, however, after impregnation with the soluble albumen salt be dipped in a dilute acid-bath or exposed to acid-vapors instead of formic aldehyde. The soluble casein salts have the peculiar property of easily penetrating the cork tissues even when employed in concentrated solutions and can be precipitated in the tissues by the natural acidity of the wine. In practice, however, it is found more advantageous to fix the casein in the impregnated corks before use by treatment with dilute organic or mineral acids or preferably with formic aldehyde. The casein thus fixed forms insoluble elastic and invisible films in the cork tissue which resist the penetration of liquids.

In order to carry out my invention, I employ, preferably, a neutral aqueous solution of the sodium salt of casein. For example, I dip the corks in a bath made by dissolving one hundred parts of casein in one thousand

parts of water with the aid of sufficient caustic soda to produce a neutral solution. The dipping is preferably carried out at a temperature of 50° centigrade, and the corks are allowed to remain in the bath for one or more hours or until cold. They are then drained and dried or dipped direct into a second bath containing a five-per-cent. solution of formic aldehyde, also preferably at 50° centigrade, for one hour and again drained and dried. The order of these baths may be reversed, or in the place of a formic aldehyde solution I may expose the corks to formic aldehyde gas.

I do not limit myself to baths of the above strength, and the temperature and time of exposure may, of course, also be varied within wide limits.

What I claim, and desire to secure by Letters Patent, is—

1. Method of treating cork stoppers consisting in impregnating the cork with a soluble casein salt.

2. Method of treating cork stoppers consisting in impregnating the cork with an alkali salt of casein.

3. Method of treating cork stoppers consisting in impregnating the cork with a sodium salt of casein.

4. Method of treating cork stoppers consisting in soaking the cork in an aqueous solution of a soluble casein salt fixing with formic aldehyde and drying.

5. Method of treating cork stoppers consisting in soaking the cork in an aqueous solution of an alkali salt of casein fixing with formic aldehyde and drying.

6. Method of treating cork stoppers consisting in soaking the cork in an aqueous solution of a sodium salt of casein fixing with formic aldehyde and drying.

7. As a new article of manufacture a casein-ated cork stopper.

In witness whereof I have hereunto signed my name in the presence of two subscribing witnesses.

HEINRICH HELBING.

Witnesses:

GEORGE BELOE ELLIS,

ROBERT MILTON SPEARPOINT.